



US010519551B2

(12) **United States Patent**  
**Yamazaki et al.**

(10) **Patent No.:** **US 10,519,551 B2**  
(45) **Date of Patent:** **Dec. 31, 2019**

(54) **ELECTRICAL STEEL SHEET**

(71) **Applicant:** **NIPPON STEEL & SUMITOMO METAL CORPORATION**, Tokyo (JP)

(72) **Inventors:** **Shuichi Yamazaki**, Tokyo (JP);  
**Masaru Takahashi**, Tokyo (JP);  
**Kazutoshi Takeda**, Tokyo (JP);  
**Hiroyasu Fujii**, Tokyo (JP); **Koji Kanehashi**, Tokyo (JP)

(73) **Assignee:** **NIPPON STEEL CORPORATION**, Tokyo (JP)

(\*) **Notice:** Subject to any disclaimer, the term of this patent is extended or adjusted under 35 U.S.C. 154(b) by 221 days.

(21) **Appl. No.:** **15/533,238**

(22) **PCT Filed:** **Dec. 22, 2015**

(86) **PCT No.:** **PCT/JP2015/085849**

§ 371 (c)(1),  
(2) Date: **Jun. 5, 2017**

(87) **PCT Pub. No.:** **WO2016/104512**

PCT Pub. Date: **Jun. 30, 2016**

(65) **Prior Publication Data**

US 2017/0335464 A1 Nov. 23, 2017

(30) **Foreign Application Priority Data**

Dec. 26, 2014 (JP) ..... 2014-266780

(51) **Int. Cl.**

**B32B 9/00** (2006.01)  
**B32B 15/04** (2006.01)

(Continued)

(52) **U.S. Cl.**

CPC ..... **C23C 22/08** (2013.01); **C23C 22/17** (2013.01); **C23C 22/20** (2013.01); **C23C 22/22** (2013.01); **C23C 22/74** (2013.01)

(58) **Field of Classification Search**

None

See application file for complete search history.

(56) **References Cited**

U.S. PATENT DOCUMENTS

3,856,568 A 12/1974 Tanaka et al.  
5,945,212 A 8/1999 Tanaka et al.

(Continued)

FOREIGN PATENT DOCUMENTS

JP 53-028375 B2 8/1978  
JP 5-078855 A 3/1993

(Continued)

OTHER PUBLICATIONS

English translation of the International Preliminary Report on Patentability and Written Opinion of the International Searching Authority (Forms PCT/IB/338, PCT/IB/373 and PCT/ISA/237) in International Application No. PCT/JP2015/085849 dated Jul. 6, 2017.

(Continued)

*Primary Examiner* — David Sample

*Assistant Examiner* — Mary I Omori

(74) **Attorney, Agent, or Firm:** Birch, Stewart, Kolasch & Birch, LLP

(57) **ABSTRACT**

An electrical steel sheet (1) includes a base material (2) of electrical steel, and an insulating film (3) formed on a surface of the base material (2). The insulating film (3) contains a phosphates of one or more selected from the group consisting of Al, Zn, Mg and Ca. The phosphate exhibits a specific peak having a top within a range of -26 ppm to -16 ppm in a solid  $^{31}\text{P}$ -NMR spectrum, and a proportion of an integrated intensity of the specific peak relative to an integrated intensity of all peaks in the solid  $^{31}\text{P}$ -NMR spectrum is 30% or more.

**4 Claims, 4 Drawing Sheets**



|                      |           |    |                   |         |  |  |
|----------------------|-----------|----|-------------------|---------|--|--|
| (51) <b>Int. Cl.</b> |           |    |                   |         |  |  |
| <i>C23C 22/08</i>    | (2006.01) | JP | 2002-317277 A     | 10/2002 |  |  |
| <i>C23C 22/20</i>    | (2006.01) | JP | 2008-303411 A     | 12/2008 |  |  |
| <i>C23C 22/22</i>    | (2006.01) | JP | 2009-155707 A     | 7/2009  |  |  |
| <i>C23C 22/74</i>    | (2006.01) | JP | 2013-536289 A     | 9/2013  |  |  |
| <i>C23C 22/17</i>    | (2006.01) | JP | 2013-249486 A     | 12/2013 |  |  |
|                      |           | WO | WO 2008/012248 A1 | 1/2008  |  |  |
|                      |           | WO | WO 2009/082088 A1 | 7/2009  |  |  |
|                      |           | WO | WO 2012/057168 A1 | 5/2012  |  |  |
|                      |           | WO | WO 2014/121853 A1 | 8/2014  |  |  |

(56) **References Cited**

## U.S. PATENT DOCUMENTS

|                  |         |                |
|------------------|---------|----------------|
| 2009/0324839 A1  | 12/2009 | Klippel et al. |
| 2013/0209789 A1  | 8/2013  | Takeda et al.  |
| 2014/0272399 A1  | 9/2014  | Böhm et al.    |
| 2014/0361230 A1  | 12/2014 | Kostler et al. |
| 2015/0368158 A1* | 12/2015 | Lemaitre ..... |
|                  |         | C21D 8/1283    |
|                  |         | 428/312.6      |

## FOREIGN PATENT DOCUMENTS

|    |               |         |
|----|---------------|---------|
| JP | 6-330338 A    | 11/1994 |
| JP | 11-131250 A   | 5/1999  |
| JP | 11-152579 A   | 6/1999  |
| JP | 2001-107261 A | 4/2001  |
| JP | 2002-047576 A | 2/2002  |
| JP | 2002-249881 A | 9/2002  |

## OTHER PUBLICATIONS

International Search Report (PCT/ISA/210) issued in PCT/JP2015/085849, dated Mar. 29, 2016.

Written Opinion (PCT/ISA/237) issued in PCT/JP2015/085849, dated Mar. 29, 2016.

Korean Office Action dated Mar. 2, 2018, for Korean Patent Application No. 10-2017-7017343.

Extended European Search Report for corresponding Application No. 15873080.4, dated Jul. 26, 2018.

Indian Examination Report issued to corresponding Indian Application No. 201717010642, dated Feb. 27, 2019, together with an English translation.

\* cited by examiner

FIG. 1



FIG. 2



FIG. 3A



1.0%

FIG. 3B



0.3%

FIG. 3C



0.1%

FIG. 3D



0.03%

FIG. 3E



0.01%

FIG. 4A



FIG. 4B



## TECHNICAL FIELD

The present invention relates to an electrical steel sheet.

## BACKGROUND ART

An electrical steel sheet is used or transported under a corrosive environment. For example, the electrical steel sheet is used in hot and humid regions or transported by sea. During the transportation by sea, a large amount of salt comes flying. Therefore, the electrical steel sheet is required to have rust resistance. To obtain the rust resistance, an insulating film is formed on the surface of the electrical steel sheet. An example of the insulating film is a chromite-based insulating film. Though the chromite-based insulating film exhibits good rust resistance, hexavalent chromium used as the raw material of the chromite-based insulating film is carcinogenic. Therefore, it is required to develop an insulating film that can be formed without using hexavalent chromium as a raw material.

Examples of the insulating film that can be formed without using hexavalent chromium as a raw material include a phosphate-based insulating film, a silica-based insulating film, and a zirconium-based insulating film (PATENT LITERATURES 1 to 12). However, with these insulating films, the rust resistance at the same level as that of the chromite-based insulating film cannot be obtained. Though the rust resistance is improved by thickening the insulating film, the weldability and the caulking property decrease more with a thicker insulating film.

## CITATION LIST

## Patent Literature

Patent Literature 1: Japanese Examined Patent Application Publication No. 53-028375

Patent Literature 2: Japanese Laid-open Patent Publication No. 05-078855

Patent Literature 3: Japanese Laid-open Patent Publication No. 06-330338

Patent Literature 4: Japanese Laid-open Patent Publication No. 11-131250

Patent Literature 5: Japanese Laid-open Patent Publication No. 11-152579

Patent Literature 6: Japanese Laid-open Patent Publication No. 2001-107261

Patent Literature 7: Japanese Laid-open Patent Publication No. 2002-047576

Patent Literature 8: International Publication Pamphlet No. 2012/057168

Patent Literature 9: Japanese Laid-open Patent Publication No. 2002-47576

Patent Literature 10: Japanese Laid-open Patent Publication No. 2008-303411

Patent Literature 11: Japanese Laid-open Patent Publication No. 2002-249881

Patent Literature 12: Japanese Laid-open Patent Publication No. 2002-317277

## Technical Problem

5 An object of the present invention is to provide an electrical steel sheet capable of obtaining good rust resistance without using hexavalent chromium as a raw material of an insulating film.

## Solution to Problem

The present inventors earnestly studied to solve the above problem. As a result, it has been revealed that good rust resistance is obtained when the phosphate exhibiting a specific peak in a solid  $^{31}\text{P}$ -NMR spectrum is contained in an insulating film. It has also been revealed that use of a coating solution containing a chelating agent is important for forming the insulating film.

10 The present inventors have reached the aspects of the present invention described below as a result of further earnest studies based on the above findings.

(1)

An electrical steel sheet, including:  
a base material of electrical steel; and

15 an insulating film formed on a surface of the base material,

wherein the insulating film contains a phosphates of one or more selected from the group consisting of Al, Zn, Mg and Ca, and

20 wherein the phosphate exhibits a specific peak having a top within a range of -26 ppm to -16 ppm in a solid  $^{31}\text{P}$ -NMR spectrum, and a proportion of an integrated intensity of the specific peak relative to an integrated intensity of all peaks in the solid  $^{31}\text{P}$ -NMR spectrum is 30% or more.

(2)

25 The electrical steel sheet according to (1), wherein a half width of the specific peak is 20 ppm or more.

(3)

30 The electrical steel sheet according to (1) or (2), wherein the insulating film contains an organic resin.

## Advantageous Effects of Invention

According to the present invention, good rust resistance can be obtained without using hexavalent chromium as the raw material of the insulating film because the phosphate exhibiting a specific peak in a solid  $^{31}\text{P}$ -NMR spectrum is contained in the insulating film. This can avoid a decrease in weldability and caulking property accompanying an increase in thickness of the insulating film.

## BRIEF DESCRIPTION OF DRAWINGS

FIG. 1 is a cross-sectional view illustrating a structure of an electrical steel sheet according to an embodiment of the present invention;

FIG. 2 is a view illustrating an example of a measurement result of a solid  $^{31}\text{P}$ -NMR spectrum;

FIG. 3A is a view illustrating an example of a test result 60 of rust resistance when a concentration of sodium chloride was 1.0 mass %;

FIG. 3B is a view illustrating an example of a test result of rust resistance when a concentration of sodium chloride was 0.3 mass %;

65 FIG. 3C is a view illustrating an example of a test result of rust resistance when a concentration of sodium chloride was 0.1 mass %;

FIG. 3D is a view illustrating an example of a test result of rust resistance when a concentration of sodium chloride was 0.03 mass %;

FIG. 3E is a view illustrating an example of a test result of rust resistance when a concentration of sodium chloride was 0.01 mass %;

FIG. 4A is a view illustrating an example of a test result of rust resistance when an insulating film was formed using a coating solution not containing a chelating agent; and

FIG. 4B is a view illustrating an example of a test result of rust resistance when an insulating film was formed using a coating solution containing a chelating agent.

## DESCRIPTION OF EMBODIMENTS

Hereinafter, an embodiment of the present invention will be described in detail referring to the accompanying drawings. FIG. 1 is a cross-sectional view illustrating a structure of an electrical steel sheet according to the embodiment of the present invention.

As illustrated in FIG. 1, an electrical steel sheet 1 according to the embodiment of the present invention includes a base material 2 of electrical steel and an insulating film 3 formed on a surface of the base material 2. The base material 2 includes a composition suitable for a grain-oriented electrical steel sheet or a non-oriented electrical steel sheet.

The insulating film 3 contains a phosphate of one or more selected from the group consisting of Al, Zn, Mg and Ca. The phosphate exhibits a specific peak having a top within a range of -26 ppm to -16 ppm in a solid  $^{31}\text{P}$ -NMR spectrum, and the proportion of the integrated intensity of the specific peak relative to the integrated intensity of all peaks in the solid  $^{31}\text{P}$ -NMR spectrum (integrated intensity ratio) is 30% or more. The half width of the specific peak is preferably 20 ppm or more. Hereinafter, M sometimes denotes Al, Zn, Mg or Ca or any combination thereof.

The insulating film 3 exhibiting the above specific peak is denser and has better rust resistance than the insulating film included in a conventional electrical steel sheet. Therefore, according to the electrical steel sheet 1, good rust resistance can be obtained without decreasing the weldability and the caulking property without using hexavalent chromium as the raw material of the insulating film 3.

The solid  $^{31}\text{P}$ -NMR spectrum can be analyzed as follows for instance. The solid  $^{31}\text{P}$ -NMR spectrum of the insulating film containing phosphate reflects a molecular structure around the P atom in the insulating film as illustrated in FIG. 2, and the position of the peak (chemical shift) and the half width of the peak depend on the molecular structure. Further, a plurality of components overlap to constitute the spectrum in some cases. In peak separation of the solid  $^{31}\text{P}$ -NMR spectrum, for example, assuming that the solid  $^{31}\text{P}$ -NMR spectrum is made by overlapping of Gauss functions, an optimization calculation is performed so as to be able to reproduce the solid  $^{31}\text{P}$ -NMR spectrum using the area fraction, the peak position, and the half width of the individual Gauss function as fitting parameters. The integrated intensity ratio, the peak position, and the half width of each component can be decided from the result of the optimization calculation. In the above manner, the integrated intensity ratio of the specific peak can be obtained.

Next, a method of manufacturing the electrical steel sheet 1 will be described. This method includes applying a coating solution composed of an M-containing polyvalent metal phosphate, a chelating agent and water to the base material of the electrical steel, and baking the coating solution. Water with a total concentration of Ca ions and Mg ions of 100

ppm or less is used as the water in the coating solution. Examples of the polyvalent metal phosphate include an aluminum monophosphate, a zinc monophosphate, a magnesium monophosphate, and a calcium monophosphate.

Hereinafter, an aluminum phosphate, a zinc phosphate, a magnesium phosphate, and a calcium phosphate represent the aluminum monophosphate, the zinc monophosphate, the magnesium monophosphate, and the calcium monophosphate respectively.

In baking the coating solution, the ends of the phosphate are crosslinked by the dehydration/condensation reaction to form an insulating film. Examples of the reaction formula of the dehydration/condensation reaction include the following. The chelating agent is described as "HO—R—OH" and the metal is described as "M".



On the other hand, when a coating solution composed of the polyvalent metal phosphate and water but not containing the chelating agent is used, the reaction of Reaction formula 1 occurs but the reactions of Reaction formula 2 to Reaction formula 4 do not occur. Therefore, in the case of using the coating solution containing the chelating agent, much more crosslinking points exist in the insulating film and higher rust resistance can be obtained than in the case of using the coating solution not containing chelating agent. With more bonds of the chelating agent, a larger number of crosslinking points exist and higher rust resistance can be obtained.

As the chelating agent, for example, an oxycarbonic acid-based, dicarboxylic acid-based or phosphonic acid-based chelating agent is used. Examples of the oxycarbonic acid-based chelating agent include a malic acid, a glycolic acid and a lactic acid. Examples of the dicarboxylic acid-based chelating agent include an oxalic acid, a malonic acid and a succinic acid. Examples of the phosphonic acid-based chelating agent include an aminotrimethylene phosphonic acid, a hydroxyethylidene monophosphonic acid, and a hydroxyethylidene diphosphonic acid.

The amount of the chelating agent contained in the coating solution is 1 mass % to 30 mass % relative to the mass of the insulating film after baking. Since the coating solution containing phosphate is acidic, Fe elutes from the base material into the coating solution while the drying of the coating solution is not completed and the coating solution is kept acidic. When Fe elutes excessively to exceed the reaction limit of the chelating agent, an iron phosphate and an iron hydroxide are generated, so that the insulating film exhibiting the specific peak cannot be obtained. This phenomenon is remarkable when the amount of the chelating agent is less than 1 mass %. Accordingly, the amount of the chelating agent is 1 mass % or more relative to the mass of the insulating film after baking. On the other hand, when the amount of the chelating agent is more than 30 mass %, the phosphate in the coating solution is less than 70 mass %, so that sufficient heat resistance cannot be obtained in the insulating film. Accordingly, the amount of the chelating agent is 30 mass % or less relative to the mass of the insulating film after baking.

The chelating agent is an active compound but, once reacted with metal, becomes stable in terms of energy and

does not exhibit sufficient activity any longer. Accordingly, to keep the activity of the chelating agent high, metal other than the metal contained in the phosphate is prevented from reacting with the chelating agent before the baking of the coating solution is completed. Therefore, it is preferable that the concentration of metal ions having high reactivity with the chelating agent in water is low. Examples of the metal ion include a Ca ion and a Mg ion. When the total concentration of the Ca ions and the Mg ions is more than 100 ppm, the activity of the chelating agent decreases. Therefore, the total concentration of the Ca ions and the Mg ions is 100 ppm or less, and more preferably 70 ppm or less. A smaller amount of alkaline-earth metal ions other than the Ca ions and the Mg ions is more preferable.

The chelating agent contains a hydroxyl group at an end, and is likely to take an association state (hydrogen bond) expressed by Reaction formula 5.



(Reaction formula 5)

When the degree of association (degree of hydrogen bond) of the hydroxyl group in the chelating agent increases, the crosslinking reactions expressed by Reaction formula 2 to Reaction formula 4 hardly occur. Therefore, the application of the coating solution is preferably performed to make the degree of association as low as possible. For example, in the case of performing application using a roller (roll coating), it is preferable to apply the coating solution while giving a shear stress to the coating solution to decrease the degree of association of the chelating agent. Decreasing the diameter of the roller and increasing the moving speed of the base material can give the shear stress suitable for releasing the association state. For example, it is preferable to use a roller having a diameter of 700 mm or less and set the moving speed of the base material to 60 m/min or more, and more preferable to use a roller having a diameter of 500 mm or less and set the moving speed of the base material to 70 m/min or more.

The baking of the coating solution is performed at a temperature of 250° C. or higher, the heating rate (first heating rate) from the temperature of the base material at the application, for example, the room temperature of about 30° C., to 100° C. is 8° C./sec or more, and the heating rate (second heating rate) from 150° C. to 250° C. is lower than the first heating rate. The temperature at the application is substantially equal to the temperature of the coating solution.

The progress of the above-described association of the chelating agent occurs no longer if the flowability of the coating solution is lost. Accordingly, to make the degree of association as low as possible, it is preferable to increase the first heating rate up to the boiling point of water (100° C.). When the first heating rate is less than 8° C./sec, the degree of association of the chelating agent rapidly increases during temperature increase to make the crosslinking reactions expressed by Reaction formula 2 to Reaction formula 4 hardly occur. Therefore, the first heating rate is 8° C./sec or more.

The crosslinking reactions of the phosphate and the chelating agent and the decomposition of the chelating agent of Reaction formula 1 to Reaction formula 4 occur in a temperature range of 150° C. to 250° C. The crosslinking reactions are carried out preferably to prevent the decomposition of the chelating agent from being excessively rapid, and the second heating rate from 150° C. to 250° C. is preferably as low as possible. Capturing of the chelating agent into the phosphate structure and the crosslinking reactions are affected by the above-described degree of

association of the chelating agent. Accordingly, when the first heating rate is high and the degree of association of the chelating agent is low, the crosslinking reaction of the phosphate and the chelating agent can be accelerated even if the second heating rate is increased. Inversely, when the first heating rate is low and the degree of association of the chelating agent is high, the crosslinking reaction of the chelating agent and the phosphate needs to be accelerated by accordingly decreasing the second heating rate. From the study by the present inventors, it has been revealed that when the first heating rate is 8° C./sec or more and the second heating rate is lower than the first heating rate, the crosslinking reaction of the phosphate and the chelating agent proceeds according to the degree of association of the chelating agent and good rust resistance can be obtained. However, when the second heating rate is excessively high, for example, more than 18° C./sec, the crosslinking is not sufficiently completed, so that good rust resistance cannot be obtained even if the first heating rate is 8° C./sec or more.

Accordingly, the second heating rate is 8° C./sec or less. On the other hand, with a lower second heating rate, the productivity becomes lower, which is remarkable at less than 5° C./sec. Accordingly, the second heating rate is preferably 8° C./sec or more.

The electrical steel sheet 1 can be manufactured through the application of the coating solution to the base material of the electrical steel and baking of the coating solution.

The coating solution may contain an organic resin. The organic resin contained in the coating solution has an action of suppressing abrasion of a punching die. Therefore, use of the coating solution containing the organic resin improves the punching workability of the electrical steel sheet. The organic resin is preferably used as a water-dispersible organic emulsion. In the case where the water-dispersible organic emulsion is used, it is more preferable that less alkaline-earth metal ions such as Ca ions, Mg ions are contained therein. Examples of the organic resin include an acrylic resin, an acrylic styrene resin, an alkyd resin, a polyester resin, a silicone resin, a fluorocarbon resin, a polyolefin resin, a styrene resin, a vinyl acetate resin, an epoxy resin, a phenol resin, an urethane resin, and a melamine resin.

Next, the action of the chelating agent will be described.

To reveal the action of the chelating agent, the present inventors measured the solid  $^{31}\text{P}$ -NMR (nuclear magnetic resonance) spectrum for the insulating film formed using the coating solution containing the chelating agent and the insulating film formed using the coating solution not containing the chelating agent. FIG. 2 illustrates an example of the measurement result of the solid  $^{31}\text{P}$ -NMR spectrum. In FIG. 2, the first or third spectrum from the top is of the insulating film formed using the coating solution containing the chelating agent (Example 1, Example 3), and the second, fourth, or fifth spectrum from the top is of the insulating film formed using the coating solution not containing the chelating agent (Reference example 2, Reference example 4, Reference example 5). The aluminum phosphate was used as the polyvalent metal phosphate contained in the coating solution in Example 1, Reference example 2 and Reference example 4, and the aluminum phosphate was used as the polyvalent metal phosphate in Example 3 and Reference example 5.

As illustrated in FIG. 2, in the insulating film formed using the coating solution not containing the chelating agent, a spectrum containing a component exhibiting a peak having a top near -30 ppm and a small half width (Reference example 2, Reference example 4), or a spectrum containing

a component exhibiting a peak having a top near +13 ppm and a large half width (Reference example 5) was obtained. On the other hand, in the insulating film formed using the coating solution containing the chelating agent in Example 1, a spectrum containing a component exhibiting a peak having a top at -23 ppm and a large half width in addition to such a component as in Reference example 2 or Reference example 4 was obtained. In the insulating film formed using the coating solution containing the chelating agent in Example 3, a spectrum containing a component exhibiting a peak having a top at -18 ppm and a large half width in addition to such a component as in Reference example 5 was obtained.

The present inventors focused on the different points in the above solid  $^{31}\text{P}$ -NMR spectrum and considered that the peak contained in the solid  $^{31}\text{P}$ -NMR spectrum greatly contributes to the improvement in rust resistance of the insulating film, and investigated the relationship between them.

Here, a method of evaluating the rust resistance will be described.

Examples of the test of evaluating the rust resistance of the electrical steel sheet include the humidity cabinet test defined in JIS K 2246 and the salt spray test defined in JIS Z 2371. However, since the corrosive environments in these tests are greatly different from the corrosive environment where the electrical steel sheet rusts, the rust resistance of the electrical steel sheet cannot be appropriately evaluated by these tests.

Hence, the present inventors studied the method capable of appropriately evaluating the rust resistance in the corrosive environment where the electrical steel sheet rusts. As a result, it has been found that the following method can appropriately evaluate the rust resistance. In this method, liquid droplets of sodium chloride solutions different in concentration are attached by 0.5  $\mu\text{l}$  to the surface of the electrical steel sheet having the insulating film and dried, and the electrical steel sheet is held in an atmosphere with constant temperature and humidity of a temperature of 50° C. and a relative humidity RH of 90% for 48 hours. A thermo-hygrometer may be used. Thereafter, the presence or absence of rust is observed, and the concentration of the sodium chloride solution with which the electrical steel sheet does not rust is identified. The rust resistance is evaluated based on the concentration of the sodium chloride solution with which the rust does not form.

More specifically, in this method, after the attachment and drying of the liquid droplets of the sodium chloride solutions, the electrical steel sheet is exposed to a moist atmosphere. Such process is similar to a corrosive environment to which the electrical steel sheet is exposed. In the corrosive environment, salt adheres to the surface of the electrical steel sheet during storage, transportation and use and then the salt deliquesces due to an increase in humidity. With a higher concentration of the sodium chloride solution, a larger amount of sodium chloride remains after drying and the rust is more likely to form. Accordingly, by making an observation while decreasing stepwise the concentration of the sodium chloride solution, and specifying the concentration where the rust does not form (hereinafter, sometimes referred to as a "limit sodium chloride concentration"), the rust resistance in the corrosive environment to which the electrical steel sheet is actually exposed can be quantitatively evaluated based on the limit sodium chloride concentration.

FIG. 3A to FIG. 3E illustrate examples of the test result by the above method. In this test, the concentration of

sodium chloride was 1.0 mass % (FIG. 3A), 0.3 mass % (FIG. 3B), 0.1 mass % (FIG. 3C), 0.03 mass % (FIG. 3D), or 0.01 mass % (FIG. 3E). As illustrated in FIG. 3A to FIG. 3E, rust was observed when the concentration of the sodium chloride was 1 mass %, 0.3 mass %, 0.1 mass %, or 0.03 mass %, and rust was not observed when the concentration of the sodium chloride was 0.01 mass %. Therefore, the limit sodium chloride concentration of the electrical steel sheet is 0.01 mass %. The present inventors have confirmed that the 10 rusting state rarely changes even when the hold time in the atmosphere with constant temperature and humidity is over 48 hours.

FIG. 4A illustrates an example of a test result by the above method about the electrical steel sheet having the insulating film formed using the coating solution not containing the chelating agent, and FIG. 4B illustrates an example of a test result by the above method about the electrical steel sheet having the insulating film formed using the coating solution containing the chelating agent. Each of the coating solutions 15 contains the aluminum phosphate as the polyvalent metal phosphate. On the electrical steel sheet having the insulating film formed using the coating solution not containing the chelating agent, rust was observed in the case of using the sodium chloride solution having a concentration of 0.03 mass % as illustrated in FIG. 4A. On the other hand, on the electrical steel sheet having the insulating film formed using the coating solution containing the chelating agent, no rust was observed even in the case of using the sodium chloride solution having a concentration of 0.2 mass % as illustrated 20 in FIG. 4B.

As described above, the limit sodium chloride concentration is higher and better rust resistance can be obtained in the case of forming the insulating film using the coating solution containing the chelating agent than in the case of forming the 25 insulating film using the coating solution not containing the chelating agent.

The effect of improving the rust resistance by addition of the chelating agent to the above coating solution can be explained in association with the solid  $^{31}\text{P}$ -NMR spectrum. 30 The insulating film of the phosphate which is formed using the coating solution not containing the chelating agent has a structure containing a simple bond expressed by the right side of Reaction formula 1. In the solid  $^{31}\text{P}$ -NMR spectrum, this structure exhibits a peak having a top about -30 ppm and a narrow width when the phosphate is crystallized, and exhibits a peak having a top near +13 ppm and a broad width when the phosphate is amorphous. On the other hand, the insulating film of the phosphate which is formed using the coating solution containing the chelating agent also includes an amorphous structure containing a complex bond expressed by the right sides of Reaction formula 2 to Reaction formula 4. In the solid  $^{31}\text{P}$ -NMR spectrum, the amorphous structure exhibits a peak having a top in -26 ppm to -16 ppm, and the half width of the peak is, for example, 35 20 ppm or more. Though details will be described later, when the proportion of the integrated intensity of the peak exhibited by the amorphous structure (specific peak) relative to the integrated intensity of all peaks in the solid  $^{31}\text{P}$ -NMR spectrum is 30% or more, good rust resistance can be obtained.

The insulating film 3 according to the embodiment of the present invention exhibits the above specific peak in the solid  $^{31}\text{P}$ -NMR spectrum. Therefore, good rust resistance can be obtained without using hexavalent chromium as the 40 raw material of the insulating film 3 by the electrical steel sheet 1. For example, the electrical steel sheet 1 exhibits sufficient rust resistance even under a high airborne salt

environment during transportation by sea or the like or under a hot and humid environment corresponding to the subtropical zone or the tropical zone. Since the insulating film 3 does not need to be formed thick, a decrease in weldability and caulking property can be avoided.

It should be noted that the above embodiment merely illustrate concrete examples of implementing the present invention, and the technical scope of the present invention is not to be construed in a restrictive manner by the embodiment. That is, the present invention may be implemented in various forms without departing from the technical spirit or main features thereof.

### EXAMPLES

Next, examples of the present invention will be described. The condition in examples is one condition example employed for confirming the feasibility and the effect of the

present invention, and the present invention is not limited to the one condition example. The present invention can employ various conditions without departing from the scope of the present invention and within achieving the object of the present invention.

The present inventors prepared coating solutions each composed of phosphate, a chelating agent, an organic resin and water listed in Table 1 and applied to both surfaces of a base material of electrical steel and baked. The total concentration (total ion concentration) of Ca ions and Mg ions contained in the water is also listed in Table 1. The application condition and the baking condition are also listed in Table 1. The first heating rate is the heating rate from 30° C. to 100° C., and the second heating rate is the heating rate from 150° C. to 250° C. The base material contained 0.3 mass % of Si, and the thickness of the base material was 0.5 mm. In Sample No. 17, an insulating film was formed using chromate in place of phosphate.

TABLE 1

| COATING SOLUTION |                                               |                    |                    |                            | TOTAL<br>ION<br>CONCENTRATION<br>(ppm) |
|------------------|-----------------------------------------------|--------------------|--------------------|----------------------------|----------------------------------------|
| SAMPLE<br>No.    | PHOSPHATE                                     | ORGANIC<br>RESIN   | CHELATING<br>AGENT | OTHER<br>MATERIAL          |                                        |
| 1                | ALUMINUM<br>PHOSPHATE                         | N/A                | N/A                | N/A                        | 50                                     |
| 2                | ALUMINUM<br>PHOSPHATE                         | ACRYLIC            | N/A                | N/A                        | 50                                     |
| 3                | ALUMINUM<br>PHOSPHATE                         | ACRYLIC            | N/A                | N/A                        | 50                                     |
| 4                | ALUMINUM<br>PHOSPHATE<br>AND *1               | ACRYLIC            | N/A                | N/A                        | 50                                     |
| 5                | ALUMINUM<br>PHOSPHATE                         | ACRYLIC            | GLUCONIC<br>ACID   | N/A                        | 120                                    |
| 6                | MAGNESIUM<br>PHOSPHATE                        | ACRYLIC            | OXALIC<br>ACID     | N/A                        | 50                                     |
| 7                | MAGNESIUM<br>PHOSPHATE                        | ACRYLIC            | PHOSPHONIC<br>ACID | N/A                        | 50                                     |
| 8                | ALUMINUM PHOSPHATE AND<br>MAGNESIUM PHOSPHATE | ACRYLIC            | CITRIC<br>ACID     | N/A                        | 50                                     |
| 9                | ALUMINUM PHOSPHATE AND<br>ZINC PHOSPHATE      | ACRYLIC<br>STYRENE | CITRIC<br>ACID     | N/A                        | 50                                     |
| 10               | ALUMINUM<br>PHOSPHATE                         | N/A                | GLUCONIC<br>ACID   | N/A                        | 50                                     |
| 11               | ALUMINUM<br>PHOSPHATE                         | ACRYLIC            | OXALIC<br>ACID     | N/A                        | 50                                     |
| 12               | MAGNESIUM<br>PHOSPHATE                        | ACRYLIC            | PHOSPHONIC<br>ACID | N/A                        | 80                                     |
| 13               | ZINC<br>PHOSPHATE                             | ACRYLIC<br>STYRENE | CITRIC<br>ACID     | N/A                        | 50                                     |
| 14               | ALUMINUM PHOSPHATE AND<br>MAGNESIUM PHOSPHATE | POLYESTER          | PHOSPHONIC<br>ACID | N/A                        | 50                                     |
| 15               | ALUMINUM PHOSPHATE AND<br>ZINC PHOSPHATE      | EPOXY              | GLUCONIC<br>ACID   | N/A                        | 50                                     |
| 16               | ALUMINUM<br>PHOSPHATE                         | ACRYLIC            | PHOSPHONIC<br>ACID | N/A                        | 50                                     |
| 17               | (MAGNESIUM<br>CHROMATE)                       | ACRYLIC            | N/A                | N/A                        | 100                                    |
| 18               | ALUMINUM<br>PHOSPHATE                         | N/A                | GLUCONIC<br>ACID   | N/A                        | 50                                     |
| 19               | ALUMINUM<br>PHOSPHATE                         | N/A                | GLUCONIC<br>ACID   | N/A                        | 50                                     |
| 20               | ALUMINUM PHOSPHATE AND<br>MAGNESIUM PHOSPHATE | N/A                | GLOCONIC<br>ACID   | FLUOROTI-<br>TANIC<br>ACID | 50                                     |

TABLE 1-continued

| 21            | ALUMINUM PHOSPHATE AND<br>MAGNESIUM PHOSPHATE | N/A                         | GLUCONIC<br>ACID  | FLUOROTI-<br>TANIC<br>ACID             | 100                                     |                                         |                        |
|---------------|-----------------------------------------------|-----------------------------|-------------------|----------------------------------------|-----------------------------------------|-----------------------------------------|------------------------|
| SAMPLE<br>No. | APPLICATION CONDITION                         |                             |                   | BAKING CONDITION                       |                                         |                                         |                        |
|               | DIAMETER<br>OF<br>ROLLER<br>(mm)              | APPLYING<br>RATE<br>(m/min) | THICKNESS<br>(μm) | FIRST<br>HEATING<br>RATE<br>(° C./sec) | SECOND<br>HEATING<br>RATE<br>(° C./sec) | ACHIEVING<br>TEMPER-<br>ATURE<br>(° C.) |                        |
| 1             | 300                                           | 80                          | 1.0               | 12                                     | 10                                      | 300                                     | COMPARATIVE<br>EXAMPLE |
| 2             | 300                                           | 80                          | 1.0               | 12                                     | 10                                      | 300                                     | COMPARATIVE<br>EXAMPLE |
| 3             | 300                                           | 80                          | 0.5               | 12                                     | 20                                      | 300                                     | COMPARATIVE<br>EXAMPLE |
| 4             | 300                                           | 80                          | 1.0               | 12                                     | 10                                      | 300                                     | COMPARATIVE<br>EXAMPLE |
| 5             | 300                                           | 80                          | 0.5               | 12                                     | 15                                      | 300                                     | COMPARATIVE<br>EXAMPLE |
| 6             | 750                                           | 80                          | 0.5               | 12                                     | 10                                      | 300                                     | COMPARATIVE<br>EXAMPLE |
| 7             | 300                                           | 50                          | 0.5               | 12                                     | 10                                      | 300                                     | COMPARATIVE<br>EXAMPLE |
| 8             | 300                                           | 80                          | 0.5               | 8                                      | 5                                       | 300                                     | COMPARATIVE<br>EXAMPLE |
| 9             | 300                                           | 80                          | 0.5               | 12                                     | 10                                      | 230                                     | COMPARATIVE<br>EXAMPLE |
| 10            | 300                                           | 80                          | 0.5               | 12                                     | 10                                      | 300                                     | INVENTION<br>EXAMPLE   |
| 11            | 300                                           | 80                          | 0.5               | 12                                     | 8                                       | 300                                     | INVENTION<br>EXAMPLE   |
| 12            | 400                                           | 60                          | 0.5               | 12                                     | 10                                      | 300                                     | INVENTION<br>EXAMPLE   |
| 13            | 300                                           | 80                          | 0.5               | 10                                     | 8                                       | 200                                     | INVENTION<br>EXAMPLE   |
| 14            | 300                                           | 80                          | 0.5               | 12                                     | 10                                      | 250                                     | INVENTION<br>EXAMPLE   |
| 15            | 300                                           | 80                          | 0.5               | 12                                     | 10                                      | 300                                     | INVENTION<br>EXAMPLE   |
| 16            | 300                                           | 80                          | 0.5               | 12                                     | 10                                      | 300                                     | INVENTION<br>EXAMPLE   |
| 17            | 500                                           | 60                          | 0.5               | 12                                     | 10                                      | 300                                     | COMPARATIVE<br>EXAMPLE |
| 18            | 300                                           | 80                          | 0.5               | 8                                      | 8                                       | 300                                     | COMPARATIVE<br>EXAMPLE |
| 19            | 300                                           | 80                          | 0.5               | 8                                      | 8                                       | 300                                     | COMPARATIVE<br>EXAMPLE |
| 20            | 300                                           | 80                          | 0.5               | 8                                      | 8                                       | 300                                     | COMPARATIVE<br>EXAMPLE |
| 21            | 500                                           | 80                          | 0.5               | 8                                      | 8                                       | 300                                     | COMPARATIVE<br>EXAMPLE |

\*1: COPOLYMER OF FLUOROETHYLENE AND ETHYLENICALLY UNSATURATED COMPOUND

Then, measurement of the solid  $^{31}\text{P}$ -NMR spectrum and evaluation of the rust resistance and the weldability of the insulating film were performed.

In the measurement of the solid  $^{31}\text{P}$ -NMR spectrum of the insulating film, the position of the peak (chemical shift), the half width of the peak, and the proportion of the integrated intensity were obtained. The results are listed in Table 2. The underlined portion in Table 2 represents that the numerical value is out of the range of the present invention.

In the evaluation of the rust resistance, a test piece was prepared from each electrical steel sheet, liquid droplets of sodium chloride solutions different in concentration were attached by 0.5  $\mu\text{l}$  to the surface of the test piece and dried, and the test piece was held in an atmosphere with constant temperature and humidity of a temperature of 50° C. and a

relative humidity RH of 90% for 48 hours. The concentrations of the sodium chloride solutions were 0.001 mass %, 0.01 mass %, 0.02 mass %, 0.03 mass %, 0.10 mass %, 0.20 mass %, 0.30 mass %, and 1.0 mass %. Thereafter, the presence or absence of rust was observed, and the limit sodium chloride (NaCl) concentration of each test piece was identified. This result is also listed in Table 2.

In the evaluation of the weldability, the welding current was 120 A, a La—W (2.4 mm  $\varphi$ ) was used as an electrode, the gap was 1.5 mm, the flow rate of an Ar gas was 6 l/min, and the clamping pressure was 50 kg/cm<sup>2</sup>, welding was performed at various welding speeds. Then, the maximum welding speed at which blow hole was not generated was specified. The result is also listed in Table 2.

TABLE 2

| MEASUREMENT RESULT OF SOLID $^{31}\text{P}$ -NMR SPECTRUM |                                                                       |                        |                                                 |                                                        |                        |                                                 |                              |                        |                                                 |
|-----------------------------------------------------------|-----------------------------------------------------------------------|------------------------|-------------------------------------------------|--------------------------------------------------------|------------------------|-------------------------------------------------|------------------------------|------------------------|-------------------------------------------------|
| SAMPLE<br>No.                                             | NEAR -30 ppm                                                          |                        |                                                 | NEAR +13 ppm                                           |                        |                                                 | -26 ppm TO -13 ppm           |                        |                                                 |
|                                                           | POSITION<br>OF PEAK<br>(ppm)                                          | HALF<br>WIDTH<br>(ppm) | PROPORTION OF<br>INTEGRATED<br>INTENSITY<br>(%) | POSITION<br>OF PEAK<br>(ppm)                           | HALF<br>WIDTH<br>(ppm) | PROPORTION OF<br>INTEGRATED<br>INTENSITY<br>(%) | POSITION<br>OF PEAK<br>(ppm) | HALF<br>WIDTH<br>(ppm) | PROPORTION OF<br>INTEGRATED<br>INTENSITY<br>(%) |
| 1                                                         | -29                                                                   | 5                      | 100                                             | NO PEAK                                                |                        | 0                                               | NO PEAK                      |                        | 0                                               |
| 2                                                         | -30                                                                   | 5                      | 100                                             | NO PEAK                                                |                        | 0                                               | NO PEAK                      |                        | 0                                               |
| 3                                                         | -30                                                                   | 5                      | 100                                             | NO PEAK                                                |                        | 0                                               | NO PEAK                      |                        | 0                                               |
| 4                                                         | -29                                                                   | 5                      | 100                                             | NO PEAK                                                |                        | 0                                               | NO PEAK                      |                        | 0                                               |
| 5                                                         | -30                                                                   | 5                      | 80                                              | NO PEAK                                                |                        | 0                                               | -25                          | 25                     | 20                                              |
| 6                                                         | NO PEAK                                                               |                        | 0                                               | +14                                                    | 30                     | 77                                              | -17                          | 30                     | 23                                              |
| 7                                                         | NO PEAK                                                               |                        | 0                                               | +13                                                    | 30                     | 82                                              | -18                          | 30                     | 18                                              |
| 8                                                         | -29                                                                   | 5                      | 80                                              | NO PEAK                                                |                        | 0                                               | -26                          | 25                     | 20                                              |
| 9                                                         | -30                                                                   | 5                      | 75                                              | NO PEAK                                                |                        | 0                                               | -24                          | 25                     | 25                                              |
| 10                                                        | -31                                                                   | 5                      | 16                                              | NO PEAK                                                |                        | 0                                               | -25                          | 25                     | 84                                              |
| 11                                                        | -30                                                                   | 5                      | 39                                              | NO PEAK                                                |                        | 0                                               | -23                          | 25                     | 61                                              |
| 12                                                        | NO PEAK                                                               |                        | 0                                               | +13                                                    | 30                     | 65                                              | -18                          | 30                     | 35                                              |
| 13                                                        | NO PEAK                                                               |                        | 0                                               | +13                                                    | 30                     | 50                                              | -16                          | 30                     | 50                                              |
| 14                                                        | NO PEAK                                                               |                        | 0                                               | +12                                                    | 30                     | 45                                              | -20                          | 30                     | 55                                              |
| 15                                                        | -31                                                                   | 5                      | 40                                              | NO PEAK                                                |                        | 0                                               | -23                          | 25                     | 60                                              |
| 16                                                        | -29                                                                   | 5                      | 35                                              | NO PEAK                                                |                        | 0                                               | -25                          | 25                     | 65                                              |
| 17                                                        |                                                                       |                        |                                                 | NOT MEASURED                                           |                        |                                                 |                              |                        |                                                 |
| 18                                                        | -30                                                                   | 5                      | 75                                              | NO PEAK                                                |                        | 0                                               | -25                          | 25                     | 25                                              |
| 19                                                        | -30                                                                   | 5                      | 87                                              | NO PEAK                                                |                        | 0                                               | -25                          | 25                     | 12                                              |
| 20                                                        | -29                                                                   | 5                      | 77                                              | NO PEAK                                                |                        | 0                                               | -24                          | 25                     | 23                                              |
| 21                                                        | -31                                                                   | 5                      | 75                                              | NO PEAK                                                |                        | 0                                               | -26                          | 25                     | 25                                              |
| SAMPLE<br>No.                                             | RUST RESISTANCE<br>LIMIT SODIUM CHLORIDE<br>CONCENTRATION<br>(mass %) |                        |                                                 | WELDABILITY<br>MAXIMUM<br>WELDING<br>SPEED<br>(cm/min) |                        |                                                 | NOTE                         |                        |                                                 |
|                                                           | 1                                                                     | 0.02                   |                                                 | 50                                                     | 50                     |                                                 | COMPARATIVE EXAMPLE          |                        |                                                 |
| 2                                                         | 0.02                                                                  |                        |                                                 | 50                                                     | 50                     |                                                 | COMPARATIVE EXAMPLE          |                        |                                                 |
| 3                                                         | 0.01                                                                  |                        |                                                 | 100                                                    | 100                    |                                                 | COMPARATIVE EXAMPLE          |                        |                                                 |
| 4                                                         | 0.03                                                                  |                        |                                                 | 50                                                     | 50                     |                                                 | COMPARATIVE EXAMPLE          |                        |                                                 |
| 5                                                         | 0.02                                                                  |                        |                                                 | 100                                                    | 100                    |                                                 | COMPARATIVE EXAMPLE          |                        |                                                 |
| 6                                                         | 0.02                                                                  |                        |                                                 | 100                                                    | 100                    |                                                 | COMPARATIVE EXAMPLE          |                        |                                                 |
| 7                                                         | 0.02                                                                  |                        |                                                 | 100                                                    | 100                    |                                                 | COMPARATIVE EXAMPLE          |                        |                                                 |
| 8                                                         | 0.02                                                                  |                        |                                                 | 100                                                    | 100                    |                                                 | COMPARATIVE EXAMPLE          |                        |                                                 |
| 9                                                         | 0.03                                                                  |                        |                                                 | 100                                                    | 100                    |                                                 | COMPARATIVE EXAMPLE          |                        |                                                 |
| 10                                                        | 0.30                                                                  |                        |                                                 | 100                                                    | 100                    |                                                 | INVENTION EXAMPLE            |                        |                                                 |
| 11                                                        | 0.20                                                                  |                        |                                                 | 100                                                    | 100                    |                                                 | INVENTION EXAMPLE            |                        |                                                 |
| 12                                                        | 0.10                                                                  |                        |                                                 | 100                                                    | 100                    |                                                 | INVENTION EXAMPLE            |                        |                                                 |
| 13                                                        | 0.10                                                                  |                        |                                                 | 100                                                    | 100                    |                                                 | INVENTION EXAMPLE            |                        |                                                 |
| 14                                                        | 0.20                                                                  |                        |                                                 | 100                                                    | 100                    |                                                 | INVENTION EXAMPLE            |                        |                                                 |
| 15                                                        | 0.30                                                                  |                        |                                                 | 100                                                    | 100                    |                                                 | INVENTION EXAMPLE            |                        |                                                 |
| 16                                                        | 0.30                                                                  |                        |                                                 | 100                                                    | 100                    |                                                 | INVENTION EXAMPLE            |                        |                                                 |
| 17                                                        | 0.30                                                                  |                        |                                                 | 100                                                    | 100                    |                                                 | COMPARATIVE EXAMPLE          |                        |                                                 |
| 18                                                        | 0.03                                                                  |                        |                                                 | 100                                                    | 100                    |                                                 | COMPARATIVE EXAMPLE          |                        |                                                 |
| 19                                                        | 0.02                                                                  |                        |                                                 | 100                                                    | 100                    |                                                 | COMPARATIVE EXAMPLE          |                        |                                                 |
| 20                                                        | 0.03                                                                  |                        |                                                 | 100                                                    | 100                    |                                                 | COMPARATIVE EXAMPLE          |                        |                                                 |
| 21                                                        | 0.03                                                                  |                        |                                                 | 100                                                    | 100                    |                                                 | COMPARATIVE EXAMPLE          |                        |                                                 |

As listed in Table 2, both of a limit sodium chloride concentration of 0.10 mass % or more and a welding speed of 100 cm/min were obtained in Samples No. 10 to No. 16 within the range of the present invention. In other words, good rust resistance and weldability were obtained.

Since the top of the peak was not in the range of -26 ppm to -16 ppm in Samples No. 1 to No. 4, the limit sodium chloride concentration was 0.03 mass % or less or the welding speed was 50 cm/min. In other words, the rust resistance or the weldability or both of them were low.

Since the top of the peak was in the range of -26 ppm to -16 ppm but the proportion of the integrated intensity was less than 30% in Samples No. 5 to No. 9, the limit sodium chloride concentration was 0.03 mass % or less. In other words, the rust resistance was low.

Since the top of the peak was in the range of -26 ppm to -16 ppm but the proportion of the integrated intensity was

less than 30% in Samples No. 18 to No. 21, the limit sodium chloride concentration was 0.03 mass % or less. In other words, the rust resistance was low.

55

#### INDUSTRIAL APPLICABILITY

The present invention is applicable, for example, in an industry of manufacturing an electrical steel sheet and an industry using the electrical steel sheet.

The invention claimed is:

1. An electrical steel sheet, comprising:  
a base material of electrical steel; and  
an insulating film formed on a surface of the base material,  
wherein the insulating film contains at least one type of  
phosphate selected from the group consisting of Al, Zn,  
Mg and Ca, and

60

65

wherein the at least one type of phosphate exhibits a specific peak having a top within a range of -26 ppm to -16 ppm in a solid  $^{31}\text{P}$ -NMR spectrum, and a proportion of an integrated intensity of the specific peak relative to an integrated intensity of all peaks in the solid  $^{31}\text{P}$ -NMR spectrum is 30% or more. 5

2. The electrical steel sheet according to claim 1, wherein a half width of the specific peak is 20 ppm or more. 10

3. The electrical steel sheet according to claim 2, wherein the insulating film contains an organic resin.

4. The electrical steel sheet according to claim 1, wherein the insulating film contains an organic resin. 15

\* \* \* \* \*